

March 9, 1926.

1,576,274

G. M. HARRIS

MANUFACTURE OF TIN PLATE

Filed March 28, 1925



INVENTOR

Gavin M. Harris  
By George, Robbins & Parmalee

His Atty

## UNITED STATES PATENT OFFICE.

GAVIN MURE HARRIS, OF LANCASHIRE, ENGLAND.

## MANUFACTURE OF TIN PLATE.

Application filed March 28, 1925. Serial No. 19,186.

*To all whom it may concern:*

Be it known that I, GAVIN MURE HARRIS, a subject of the King of England, residing at Lancashire, England, have invented certain new and useful Improvements in the Manufacture of Tin Plate, of which the following is a specification.

This invention consists of improvements in or relating to the manufacture of tin-plate, the main objects being to minimize wastage and to produce a better plate.

In the method commonly practised, bars of very mild steel are heated and rolled. They are then "matched" in pairs, reheated, 15 rolled, and doubled; re-heated, rolled, opened (i. e. separated from one another) and doubled; re-heated, rolled and allowed to cool. Each piece (set of plates rolled together) contains eight plates, say 20 inches 20 wide and about 60 inches long. The pieces are then cut to the required measurements by shears, then the plates are pulled apart by hand.

The next operations are "black pickling," 25 in which the plates are immersed in hot dilute sulphuric acid, and "swilling," in which they are washed with cold running water. The plates are then sorted by hand to remove those plates which have not been 30 sufficiently attacked by the acid. These are returned for further pickling.

The next step in the existing method, known as "black packing," consists in packing the plates while still wet in piles on the 35 annealing stands. An annealing cover (an inverted rectangular box made of steel or wrought-iron) is placed over each pile of plates, the space between this cover and the lip of the stand being filled with sand. The 40 plates are then subjected to the process known as "black annealing," in which the pots (stand, cover and plates inside) are heated to a temperature sufficiently high to ensure softening. The pots are removed 45 from the furnace and allowed to cool before the covers are taken off, after which the plates are "thrown out" by subjecting the piles of plates to repeated blows from sledge hammers (or pneumatic hammers) to separate 50 the plates one from another. The plates are then cold rolled to impart the requisite finish to the surface. The cold

rolling hardens the plates somewhat, and they are therefore annealed once more in the process of "white annealing." It is not necessary in the second annealing to heat to so high a temperature nor for such a long time as in the first.

The plates are now subjected to the process of "white pickling," generally in weaker sulphuric acid than was used in the previous pickling; then they are swilled and are immersed in water preparatory to tinning.

One feature of the present invention comprises a modification in the manufacture of tin-plate wherein black-pickling is carried out after black annealing and the plates when pickled and swilled are dried at a temperature not exceeding 100° C. (preferably by absorption) and directly passed to the cold-rolling plant. Preferably the black annealing follows directly upon the hot rolling, shearing and opening operations. The order of the steps of black annealing and 65 pickling is thus inverted and this inversion has many advantages. All oxidation is removed before the plate goes through the cold rolling process. In the old method, plates oxidized too severely during black annealing had to be returned to the pickling for the purpose of removing the oxidation, and then re-annealed.

In the ordinary process of manufacture the annealing step serves two functions; it not only softens the plates, but also serves to dry them after pickling, and the advantage of using the annealing step for drying is that unlike drying by heating the plates at low temperatures, serious oxidation of the plates is avoided, at all events in the case of those plates which have been subjected to sufficient superincumbent weight to keep them piled close together so that air is excluded from the surfaces on cooling. However, the upper plates of the pile, which get less weight on them, are oxidized and have to be returned for black pickling again. In the ordinary process they are then re-annealed. By the present process "returns" 85 and their re-treatment can be avoided altogether. The present invention also contemplates the treatment of the "returns" in the ordinary process after their second black 90 annealing. The present invention also contemplates the treatment of the "returns" in the ordinary process after their second black 95 annealing. The present invention also contemplates the treatment of the "returns" in the ordinary process after their second black 100 annealing.

pickling, and in this case they are dried and passed directly to the cold rolling plant without re-annealing. Their mechanical properties are superior to those of re-annealed plates.

The importance of avoiding oxidation during drying is very great as otherwise the cold rolling process will roll oxide into the metal and spoil the surface. It has now 10 been found that in drying by evaporation oxidation tends to occur. The moisture is according to this invention removed by absorption into a suitable absorbent medium applied to the plates. In a preferred process the plates are dried by bringing water absorbent material into contact with the surfaces of the plates, removing it, heating it to drive off the absorbed water, and re-applying it continuously to fresh plate-surfaces.

The following is a description by way of example of one method of carrying this invention into effect:—

After the steps of hot rolling in the mills, 25 shearing and opening, the plates are subjected to the steps of black packing, black annealing and throwing out (i. e. separating the plates).

Pickling and drying are then effected 30 and the accompanying drawing illustrates diagrammatically one suitable form of apparatus for this purpose:—

The separated plates are placed on a table A in a pile. An oscillating arm B provided with a sucker C (connected with a suitable source of suction) is so pivoted that it can lift the plates one at a time from the table A and deposit them in the position indicated by chain lines on an inclined guide

40 D. Suitable known means are provided for keeping the sucker wet so that its suction is maintained. From the guide D the plates slide into the pickling vat E containing hot dilute sulphuric acid through which they are

45 fed by wheels F provided on their periphery with feeding-snugs f. The wheels F are rotated at such a speed that the plates remain in the pickling vat for the required time. On emerging from it they enter the nip of a pair of rubber-covered feed rolls G and pass between water sprays H so that they are swilled to remove acid.

The rolls G, of which there are several pairs, act in conjunction with a guide g to 55 direct the plates into a water bath K through which they are conveyed by a second arrangement of feed wheels F and delivered by further rolls G to drying rollers L.

60 The drying rolls L are covered on their external surface with a thick layer l of porous absorbent material, such as felt. Through a suitable trunnion at one end steam is admitted to the interior of the rolls 65 and the felt is maintained at a temperature

of about 100° C. After passing through two pairs of drying rollers L, the plates enter a further pair of feed rolls M and are deposited on a conveyor N which removes them from the apparatus.

In operation the oxidation upon the plates is removed by the acid. The plates are then swilled. In the water-bath they are washed and the water contains a small percentage of some chemical which has the property of precipitating colloidal ferric hydroxide, such e. g. as potassium bichromate. On entering the drying rolls their moisture is removed by absorption before it has had any opportunity to cause oxidation of the plates. 70 The moisture is then evaporated from the felt by reason of the heat of the latter, and the felt on coming again into contact with a plate, after a revolution of the drying roll L, is sufficiently dry to continue to absorb 75 moisture effectively. The plates are thus dried without ever reaching a temperature as high as 100° C. and without any evaporation taking place from them.

Various modifications may be made in the drying arrangements, for example instead of simply having rollers covered with absorbent material, a band of such material may be caused to pass over a pair or more of rollers on each side of the plates and the bands may be in contact with the plates for a considerable distance. Instead of felt, other absorbent material may be used and this may be in the form of a rope wound closely around the drying rolls. The means for feeding the plates through the baths E and K may vary. The pickling bath E is heated as usual, and any desired or suitable means for this purpose or for heating the drying rolls may be employed. In practice the machine would be made sufficiently wide to receive a number of plates simultaneously side by side.

What I claim as my invention and desire to secure by Letters Patent is:—

1. A process for the manufacture of tin-plate which comprises in combination the stages of hot rolling the plates, thereafter black annealing them, then black pickling and swilling them, thereafter drying them in such manner that they do not reach a temperature substantially exceeding 100° C., thereafter passing the plates as dried to the cold-rolling plant and cold rolling them, then preparing the plates for tinning, and tinning them.

2. A process for the manufacture of tin-plate which comprises in combination the stages of hot rolling the plates, thereafter black annealing them, then black pickling and swilling them, thereafter drying them by bringing water-absorbent material into contact with the surfaces of the plates, removing it, heating it to drive off the absorbed water and reapplying it continuously

- to fresh plate-surfaces, thereafter passing the plates as dried to the cold-rolling plant and cold rolling them, then preparing the plates for tinning, and tinning them.
5. 3. A process for the manufacture of tin-plate which comprises in combination the stages of hot-rolling, shearing and opening the plates, thereafter, without any intermediate operation, black annealing them, then black pickling and swilling them, thereafter drying them in such manner that they do not reach a temperature substantially exceeding 100° C., thereafter passing the plates as dried to the cold-rolling plant 70 and cold rolling them, then preparing the plates for tinning, and tinning them.
10. 4. A process for the manufacture of tin-plate which comprises in combination the stages of hot-rolling, shearing and opening the plates, thereafter, without intermediate 75 operation, black annealing them, then black pickling and swilling them, thereafter drying them by bringing water-absorbent material into contact with the surfaces of the plates, removing it, heating it to drive off the absorbed water and reapplying it continuously to fresh plate-surfaces, thereafter passing the plates as dried to the cold-rolling plant and cold rolling them, then preparing the plates for tinning, and tinning them.
15. 5. A process for the manufacture of tin-plate which comprises in combination the stages of hot-rolling the plates, thereafter 80 black annealing them, then black pickling and swilling them, treating the plates with a wash solution containing potassium bichromate, thereafter drying them by bringing water-absorbent material into contact with the surfaces of the plates, removing it, heating it to drive off the absorbed water and reapplying it continuously to fresh plate-surfaces, thereafter 85 passing the plates as dried to the cold-rolling plant and cold-rolling them, then preparing the plates for tinning, and tinning them.
20. 6. A process for the manufacture of tin-plate which comprises in combination the stages of hot-rolling the plates, thereafter black annealing them, then black pickling and swilling them, thereafter drying them by bringing water-absorbent material into contact with the surfaces of the plates, removing it, heating it to drive off the absorbed water and reapplying it continuously to fresh plate-surfaces, thereafter 90 passing the plates as dried to the cold-rolling plant and cold rolling them, then preparing the plates for tinning, and tinning them.
25. 7. A process for the manufacture of tin-plate which comprises in combination the stages of hot-rolling the plates, thereafter black annealing them, then black pickling and swilling them, treating the plates with a wash solution containing a solute which precipitates colloidal ferric hydroxide, thereafter drying them in such manner that they 95 do not reach a temperature substantially exceeding 100° C., thereafter passing the plates as dried to the cold-rolling plant and cold rolling them, then preparing the plates for tinning, and tinning them.
30. 8. A process for the manufacture of tin-plate which comprises in combination the stages of hot-rolling the plates, thereafter black annealing them, then black pickling and swilling them, thereafter bringing them into contact with absorbent drying webs supported upon rollers which are internally steamheated, thereafter passing the plates as dried to a cold rolling plant and cold-rolling them, preparing the plates for tinning, and tinning them.
35. 9. A process for the manufacture of tin-plate which comprises in combination the stages of hot-rolling the plates, thereafter black annealing them, then black pickling and swilling them, thereafter bringing them into contact with absorbent drying webs supported upon rollers which are internally steamheated, thereafter passing the plates as dried to a cold rolling plant and cold-rolling them, preparing the plates for tinning, and tinning them.
40. 10. A process for the manufacture of tin-plate which comprises in combination the stages of hot-rolling, shearing and opening the plates, thereafter, without any intermediate operation, black annealing them, then black pickling and swilling them, treating the plates with a wash solution containing a solute which precipitates colloidal ferric hydroxide, thereafter bringing them into contact with absorbent drying webs supported upon rollers which are internally steamheated, thereafter passing the plates as dried to a cold-rolling plant and cold-rolling them, preparing the plates for tinning, and tinning them.
45. 11. Apparatus for drying sheet metal which comprises in combination means to receive plates and feed them automatically in a direction parallel to the plate surfaces and continuous drying webs of water absorbent material so disposed as to be in contact with both sides of the plates when in use to absorb moisture therefrom, means to move the drying webs so as to present continuously a fresh part of the web surfaces
50. 12. A process for the manufacture of tin-plate which comprises in combination the stages of hot-rolling, shearing and opening the plates, thereafter, without any intermediate operation, black annealing them, then black pickling and swilling them, thereafter drying them by bringing water-absorbent material into contact with the surfaces of the plates, removing it, heating it to drive off the absorbed water and reapplying it continuously to fresh plate-surfaces, thereafter passing the plates as dried to the cold-rolling plant and cold rolling them, then preparing the plates for tinning, and tinning them.
55. 13. A process for the manufacture of tin-plate which comprises in combination the stages of hot-rolling the plates, thereafter black annealing them, then black pickling and swilling them, treating the plates with a wash solution containing a solute which precipitates colloidal ferric hydroxide, thereafter drying them by bringing water-absorbent material into contact with the surfaces of the plates, removing it, heating it to drive off the absorbed water and reapplying it continuously to fresh plate-surfaces, thereafter passing the plates as dried to the cold-rolling plant and cold rolling them, then preparing the plates for tinning, and tinning them.
60. 14. A process for the manufacture of tin-plate which comprises in combination the stages of hot-rolling the plates, thereafter black annealing them, then black pickling and swilling them, treating the plates with a wash solution containing a solute which precipitates colloidal ferric hydroxide, thereafter drying them by bringing water-absorbent material into contact with the surfaces of the plates, removing it, heating it to drive off the absorbed water and reapplying it continuously to fresh plate-surfaces, thereafter passing the plates as dried to the cold-rolling plant and cold rolling them, then preparing the plates for tinning, and tinning them.
65. 15. A process for the manufacture of tin-plate which comprises in combination the stages of hot-rolling, shearing and opening the plates, thereafter, without any intermediate operation, black annealing them, then black pickling and swilling them, thereafter drying them by bringing water-absorbent material into contact with the surfaces of the plates, removing it, heating it to drive off the absorbed water and reapplying it continuously to fresh plate-surfaces, thereafter passing the plates as dried to the cold-rolling plant and cold rolling them, then preparing the plates for tinning, and tinning them.

thereto and means to heat the webs to a temperature sufficient to evaporate absorbed moisture therefrom while out of contact with the plates.

- 5 12. In apparatus for drying sheet metal the combination of feed rollers to advance the plates through the apparatus and ro-

tatable drying rollers in contact with the plates consisting of steam-heated cylinders covered on their exterior surface with yielding water-absorbent material. 10

In testimony whereof I affix my signature.

**GAVIN MURE HARRIS.**